

## UNITED STATES PATENT OFFICE

2,312,199

## TREATMENT OF CELLULOSIC TEXTILE MATERIALS

Ernest Edward Tallis and Wilfred John Charles Field, Coventry, England, assignors to Courtaulds Limited, London, England, a British company

No Drawing. Application October 8, 1940, Serial No. 360,340. In Great Britain November 22, 1939

5 Claims. (Cl. 106—164)

This invention relates to the treatment of cellulosic textile materials for the purpose of improving their affinity for those dyestuffs commonly used for dyeing wool and the like animal fibres.

It has already been proposed to improve the affinity of cellulosic textile materials for acid wool dyestuffs by incorporating therein products obtained by the interaction of aryl isocyanates or isothiocyanates with ethylene imine, its homologues or polymers, or with proteins dissolved in ethylene imine or its homologues or polymers, or with proteins dissolved in or reacted with nitrogenous bases. It has also been proposed to incorporate alkyl polyamines in cellulosic textile materials for the same purpose.

We have now found that compounds obtained by the action of an aryl isocyanate and/or aryl isothiocyanate on a polyalkylene poly amine can be incorporated in cellulosic materials for the purpose of facilitating the dyeing of these materials with those dyestuffs commonly used for dyeing wool and the like animal fibres.

The polyalkylene polyamine which can be used to combine with the aryl isocyanate and/or aryl isothiocyanate is a compound such as ethylene diamine  $\text{NH}_2\text{CH}_2\text{CH}_2\text{NH}_2$ , trimethylene diamine  $\text{NH}_2\text{CH}_2\text{CH}_2\text{CH}_2\text{NH}_2$ , triethylene tetramine

$\text{NH}_2\text{CH}_2\text{CH}_2\text{NH} \cdot \text{CH}_2\text{CH}_2\text{NH} \cdot \text{CH}_2\text{CH}_2\text{NH}_2$   
tetraethylene pentamine

$\text{NH}_2\text{CH}_2\text{CH}_2(\text{NHCH}_2\text{CH}_2)_3\text{NH}_2$

and pentaethylene hexamine

$\text{NH}_2\text{CH}_2\text{CH}_2(\text{NHCH}_2\text{CH}_2)_4\text{NH}_2$

or other member of the series

$\text{NH}_2\text{C}_2\text{H}_4(\text{NHC}_2\text{H}_4)_n\text{NH}_2$

where  $n$  is an integer, or also a compound obtained from any of the aforesaid bodies by further alkylation, for instance by condensation with an aliphatic alkylating agent containing more than one alkylating group in the molecule, for example, alpha-dichlorhydrin

$(\text{CH}_2\text{Cl} \cdot \text{CHOH} \cdot \text{CH}_2\text{Cl})$

dichlorethylene, trimethylene bromide, dichlor-isopropyl ether, triglycol dichloride or symmetrical dichloracetone, or by condensation with an alkylene oxide, for example, ethylene oxide.

The compounds derived from the action of an aryl isocyanate and/or isothiocyanate on a simple polyalkylene polyamine, such as ethylene diamine or diethylene triamine, confer a relatively

weak affinity for the said dyestuffs on cellulosic materials with which they are incorporated. The more complex polyamines, however, give reaction products with the said isocyanates and/or isothiocyanates which confer an affinity for the said dyestuffs on cellulosic materials more closely resembling that possessed by wool.

When dyeing with strong acid wool dyestuffs a good effect can be obtained if the isocyanate and/or isothiocyanate reaction product as above described be treated either before or after incorporation in the cellulosic material with a halogenating agent such for instance as chlorine or bromine, or a hypochlorite or hypobromite, as this tends to prevent the dye from wandering from the cellulose to other admixed textiles during any prolongation of the dyeing treatment. The treatment with the halogenating agent can be combined with a bleaching treatment of the material, should such bleaching be necessary, by immersing the material in a dilute solution of sodium hypochlorite.

The isocyanate and/or isothiocyanate reaction products according to the present invention may be incorporated in the cellulosic textile material in any convenient manner, for example, by impregnating the material with a solution or dispersion thereof. In the case of artificial threads, for instance those produced from viscose, we prefer to add a solution or dispersion of the reaction product to the spinning solution from which the artificial threads are made.

The following examples illustrate how the said invention may be carried out in practice although the invention is not restricted to these examples. The parts are by weight.

## Example 1

44 parts of a 70 per cent aqueous solution of triethylene tetramine are condensed with 52 parts of anhydrous alpha-dichlorhydrin

$(\text{CH}_2\text{Cl} \cdot \text{CHOH} \cdot \text{CH}_2\text{Cl})$

to give an aqueous solution containing approximately 56 per cent of polyamine. 34 parts of this polyamine solution diluted with 700 parts of water and  $\frac{1}{2}$  part of an emulsifying agent such for instance as propyl naphthalene sulphonic acid are reacted with 45 parts of phenyl-isothiocyanate in a pebble mill as described in British Patent Specification No. 536,687. The dispersion obtained is mixed with 1,400 parts of viscose which is formed into threads in known manner. The resulting threads or fabric made therefrom have an enhanced affinity for those dyestuffs

commonly used for dyeing wool and the like animal fibres.

*Example 2*

This is carried out as in Example 1 and in addition the resulting threads are desulphurised and bleached in a 0.3 per cent solution of sodium hypochlorite. Excess hypochlorite is destroyed with dilute sulphuric acid and the threads are washed and dried. The resulting threads or fabric made therefrom have a good affinity for strong acid wool dyestuffs and there is a very little tendency for the dye to migrate if other textiles are also present during a boiling operation.

*Example 3*

3 parts of tetraethylene pentamine are heated to approximately 100° centigrade and then, while agitating, ethylene oxide is passed in under a pressure of six inches of mercury until 1 part of ethylene oxide has been absorbed. 1 part of the compound thus obtained is dissolved in 3 parts of benzyl alcohol and 2 parts of phenyl isothiocyanate are slowly added while cooling. 2 parts of the solution obtained are dispersed in 170 parts of viscose which is spun into a bath containing:

|                   | Parts |
|-------------------|-------|
| Sulphuric acid    | 8½    |
| Glucose           | 9     |
| Ammonium sulphate | 4     |
| Sodium sulphate   | 12    |
| Zinc sulphate     | 1     |
| Water             | 65½   |

The threads are then washed, desulphurised and bleached. The resulting fibre has a good affinity for those dyestuffs commonly used for dyeing wool and the like animal fibres.

What we claim is:

1. A process for improving the affinity of cellulosic textile material for those dyestuffs commonly used for dyeing wool and the like animal fibres, which comprises incorporating in the said material a compound obtained by condensing a compound selected from the group consisting of aryl isocyanates and aryl isothiocyanates with a polyalkylene polyamine.
- 5 2. A process as claimed in claim 1, in which the polyalkylene polyamine is condensed with an aliphatic alkylating agent containing more than one alkylating group in the molecule before reaction with a compound selected from the group consisting of aryl isocyanates and aryl isothiocyanates.
- 10 3. A process as claimed in claim 1, in which the polyalkylene polyamine is condensed with ethylene oxide before reaction with a compound selected from the group consisting of aryl isocyanates and aryl isothiocyanates.
- 15 4. A process for improving the affinity of cellulosic textile material for strong acid wool dyestuffs which comprises incorporating in the material a compound obtained by condensing a compound selected from the group consisting of aryl isocyanates and aryl isothiocyanates with a polyalkylene polyamine, the said compound being treated with a halogenating agent either before or after the said incorporation.
- 20 5. A process as claimed in claim 1, in which a solution or dispersion of the reaction product obtained by condensing a compound selected from the group consisting of aryl isocyanates and aryl isothiocyanates with a polyalkylene polyamine is added to viscose.

ERNEST EDWARD TALLIS.

WILFRED JOHN CHARLES FIELD.